

## UNITED STATES PATENT OFFICE

2,334,230

## GOLDBEATER'S FOIL

Donald D. Swift, Hartford, Conn., assignor to M. Swift & Sons, Inc., a corporation of Connecticut

No Drawing. Application October 28, 1939,  
Serial No. 301,796

3 Claims. (Cl. 29—17)

My present invention relates to the goldbeater's art and more particularly to an improved goldbeater's foil.

When gold or other precious base metal is beaten into thin metallic sheets, it is first rolled into a ribbon, the usual thickness of the ribbon being about  $\frac{1}{1000}$  of an inch. This ribbon is cut into squares approximately  $1\frac{1}{8}$  inches in width and the squares are filmed between membranes known as cutch paper, the trade name for a special paper made from ground animal hide. After the squares have been filmed between these papers, the resulting packet is beaten until the initial squares have spread to the full size of the cutch paper, about four inches in width. These expanded squares of metal are removed from the paper squares and are quartered, and the quartered squares are in turn filmed between membranes known as the goldbeater's skin to provide a packet form which is again beaten, each square now spreading to a diameter of about  $5\frac{1}{2}$  inches. These squares are again quartered and the process is repeated until the quartered squares become approximately six inches in diameter, the shape being somewhat irregular. These squares are preferably again quartered, filmed and beaten. Specially prepared membranes of animal origin are used for this purpose, these membranes being very expensive, and having certain recognized disadvantages in use, the principal disadvantage resulting from an unavoidable retention of fat content in the course of their preparation; the fat content makes their direct use for thin (shoder or mold) beating inadvisable, and they are therefore first used for thick (cutch) beating before they can be effectively used for thin beating. Furthermore, goldbeater's skin is not smooth, is not of uniform thickness, stretches about 3 or 4% under beating, is not uniformly tough in all directions, tends to split, and is hygroscopic, wherefore the quality of the beaten leaf depends largely upon the weather conditions during beating.

These disadvantages are effectively overcome by my present invention. I replace the animal goldbeater's skin for interleaving the metallic leaf during beating with foils of cellulose acetate in sheet form, the thickness of the cellulose acetate sheet being between .008 to .030 inch, and preferably .01 inch, which is approximately the thickness of goldbeater's skin. I have found that cellulose acetate mixtures are ideally suited for the described purpose. The commercial cellulose acetate is, however, mixed with a plasticizer or a plurality of plasticizers in varying percentages;

and I have found that the plasticizer, if present in excess quantity, tends to adversely affect the lubricant used with the goldbeater's skin during the beating operation. Inasmuch as a plasticizer is essential, I have discovered that a plasticizer such as tricresyl phosphate when used with the commercial cellulose acetate in quantities of between 8 to 10% gives the most satisfactory results. Other plasticizers or a plurality of plasticizers may also be found suitable; however, I prefer to keep the total percentage of plasticizer below 10%.

These foils, if desired, may be brushed or otherwise provided with any of the lubricating or "gut" preparations commonly employed as coatings for goldbeater's skin, consisting essentially of isinglass, gum arabic, shellac, and spices such as saffron, cinnamon, and cloves in red wine. However, the cellulose acetate foil may be used to advantage without such a coating. For example, I have found that aluminum foils may be beaten with cellulose acetate foils without the use of any lubricating or "doctoring" material. On the other hand, for best results, I have found that a lubricant is preferable for goldbeating. A preferred lubricant is disclosed in my copending application entitled Goldbeater's lubricant, filed October 28, 1939, Serial No. 301,797.

I have found that the use of the cellulose acetate as the goldbeater's skin will reduce the beating time of the gold approximately  $\frac{1}{3}$  as compared with the use of standard goldbeater's skin. Furthermore, beating with cellulose acetate foils gives the gold a very flat surface and a high initial burnishing. Inasmuch as the cellulose acetate with the 8 to 10% plasticizer will retain its elasticity under beating it can be immediately used for thin beating as it does not give or stretch. The gold will have a substantially flat and uniform thickness. The cellulose acetate foils can be obtained in a more uniform thickness than goldbeater's skin, will not stretch under use, and is non-splitting and uniformly tough in all directions.

Furthermore, the cellulose acetate is extremely cheap, is devoid of fat so that the foils can immediately be employed for mold beating, and is non-hygroscopic.

The durability of these new foils, that is their resistance to hammer blows, is superior to that of goldbeater's skin, and far superior to other substitutes that have been utilized such as Cellophane and the like. For example, I have found that Cellophane is hygroscopic in character and will crack if dehydrated. Therefore, the applica-

tion of a lubricant on Cellophane causes moisture in the Cellophane to affect the lubricant, or vice versa, and thus give indeterminate results. While cellulose acetate with approximately 8% plasticizer will retain its elasticity under constant beating, Cellophane and heavily plasticized cellulose acetate does not do so. Cellulose acetate also provides a better surface finish than Cellophane because of inherent surface conditions imposed during the process of manufacture, the cellulose acetate being made on highly polished rolls.

Although cellulose acetate has been found preferable for the above described use, due to its physical characteristics and its low cost, other chemical compositions of similar physical nature may also be used, examples being ethyl cellulose, cellulose nitrates, styrene resins, methyl methacrylate resins, vinyl chloride acetates, and phthalates such as propyl and methyl. The amount of plasticizer or softener used should be calculated or determined to obtain a predetermined plasticity which will not permit the foil to permanently stretch under the hammer beating and produce a bulged center.

While I have described a specific material for 25

use as a goldbeater's skin, it is obvious that other materials and mixtures of materials having similar physical and chemical characteristics may be used instead with various other plasticizers, within the spirit and scope of the invention as defined in the appended claims.

I claim:

1. A foil for metal beating comprising a sheet of cellulose acetate and tricresyl phosphate plasticizer, the percentage of plasticizer being below 10 per cent, and the thickness of the sheet being from .008 to .030 inch.

2. A metal beating packet comprising layers of material adapted to receive metal foils therebetween, said material comprising cellulose acetate and tricresyl phosphate plasticizer, the thickness of the layers being from .008 to .030 inch.

3. A metal beating packet comprising layers of material adapted to receive metal foils therebetween, said material comprising cellulose acetate and tricresyl phosphate plasticizer, the percentage of plasticizer being below 10 per cent, the thickness of the layers being from .008 to .030 inch.

DONALD D. SWIFT,